

# UNITED STATES PATENT OFFICE.

CLEMENT L. PERKINS, OF PITTSBURGH, PENNSYLVANIA, ASSIGNOR TO METALS  
RECOVERY COMPANY, OF NEW YORK, N. Y., A CORPORATION OF MAINE.

## FLOTATION OF MINERALS.

1,322,816.

Specification of Letters Patent. Patented Nov. 25, 1919.

No Drawing.

Application filed July 2, 1919. Serial No. 308,321.

To all whom it may concern:

Be it known that I, CLEMENT L. PERKINS, a citizen of the United States, residing at Pittsburgh, in the county of Allegheny, 5 State of Pennsylvania, have invented certain new and useful Improvements in the Flotation of Minerals; and I do hereby declare the following to be a full, clear, and exact description of the invention, such as will 10 enable others skilled in the art to which it appertains to make and use the same.

This invention relates to the concentration of minerals, such as sulfid ores and the like, (for example, chalcopyrite with a siliceous gangue), by flotation, and is based 15 upon the discovery that improved results can be obtained by carrying out the flotation operation with the addition to the ore or mineral pulp of toluidin, either alone or 20 with the addition of other agents promoting the flotation.

The toluidin may be used in the form of a mixture of the individual toluidins, for example, of the para-toluidin and ortho-toluidin; or the individual ortho-toluidin or 25 para-toluidin can be used alone:

In using the toluidin it may be added to the ore either alone or in admixture with other agents promoting the flotation, in any 30 suitable manner, so that it will be thoroughly and uniformly distributed throughout the ore pulp. The mixture is then subjected to a flotation operation as in an ordinary Callow cell or in apparatus where 35 the air is incorporated in the ore pulp by mechanical agitation. With some ore pulps it may be desirable to add either small amounts of acids or of alkalis, depending upon the nature of the ore pulp to be treated, but in general free acid should not be 40 present to any appreciable extent when the toluidin is added.

With some ore pulps it is important not only to have no free acid present, but to add 45 sufficient free alkali to give a distinct alkaline reaction to the ore pulp during the flotation operation. Small amounts of caustic alkali, such as sodium hydrate, or of alkali salts, such as sodium carbonate, may thus 50 be added, in regulated amounts, to give the ore pulp the proper degree of alkalinity.

The amount of toluidin used may vary somewhat, for example, between one-half pound or less and one and one-half pounds

per ton of ore (that is, calculated on the weight of the ore and not of the ore pulp).

The invention will be further illustrated by the following specific example: 500 parts by weight of ore was ground in the ball or pebble mill with 250 parts of water, sodium 60 hydroxid in amount equivalent to two pounds per ton of ore, and commercial mixed toluidin equivalent to one pound per ton of ore. The resulting pulp was placed in a Callow pneumatic rougher cell, together with sufficient water to form a free-flowing pulp, and then subjected to a flotation treatment. The ore treated contained about 1.42 per cent. of copper. The concentrates produced contained about 15.4 per cent. of copper, and the recovery of the copper was 70 about 87 per cent. The ore treated was a Utah copper ore.

With ores of the character above referred to, the use of alkali is not necessary, but its 75 use has been found to greatly improve the recovery.

Comparative results obtained with the use of ortho-toluidin or para-toluidin, and mixed toluidin, composed mainly of the 80 ortho and para-toluidin, carried out in a manner similar to the specific example given above, gave the following result:

|                     | Heads. | Concts. | Recovery. |
|---------------------|--------|---------|-----------|
| Orthotoluidin.....  | 1.38   | 13.7    | 73.2      |
| Paratoluidin.....   | 1.38   | 19.9    | 86.4      |
| Mixed toluidin..... | 1.38   | 16.5    | 81.4      |

It is characteristic of the invention that 90 the froth obtained is readily broken up and the toluidin recovered therefrom so that it is available for use in the treatment of further amounts of ore. That is to say, the circuit water recovered from the concentrate 95 and even that recovered from the tailings contains notable amounts of the toluidin which can thus be returned to the process with resulting economy in the amount required to be added for subsequent operations. 100

The toluidin may be used alone to promote the flotation operation and high grades of concentrates obtained; and the resulting concentrates can be much more easily separated by filtration than the common concentrates 105 obtained by the use of oil as the flotation agent. The action of the toluidin may, however, be modified or supplemented by adding

other agents (such as oils or non-oleaginous agents) which promote the flotation and which do not prejudicially affect the action of the toluidin.

- 5 5. In applying the toluidin, it may be introduced into the tube mill in which the ore is being ground, or it may be otherwise introduced into the ore pulp in any suitable way, as, for instance, by dropping it into the ore
- 10 10. pulp before it enters the flotation cell, or by first digesting it in hot water and mixing the product with the ore pulp just before it enters the flotation cell.

What I claim is:

- 15 15. 1. The method of effecting the concentration of minerals by flotation, which comprises adding to the mineral pulp a small amount of toluidin, and subjecting the resulting mixture to a flotation operation; substantially as described.
- 20 2. The method of effecting the concentration of minerals by flotation, which com-

prises adding to the mineral pulp a small amount of toluidin and other agents promoting the flotation, and subjecting the resulting mixture to a flotation operation; substantially as described.

3. The method of effecting the concentration of minerals by flotation, which comprises adding to the mineral pulp a small amount of toluidin and sufficient alkali to give the ore pulp a distinct alkaline reaction, and subjecting the resulting mixture to a flotation operation; substantially as described.

4. The method of effecting the concentration of minerals by flotation, which comprises adding to the mineral pulp a small amount of toluidin and of oil, and subjecting the resulting mixture to a flotation opera- 40

tion; substantially as described.

In testimony whereof I affix my signature.

CLEMENT L. PERKINS.